

Patented Dec. 22, 1925.

1,566,384

# UNITED STATES PATENT OFFICE.

HENRY DREYFUS, OF LONDON, ENGLAND.

## MANUFACTURE OF ARTIFICIAL SILK AND THE LIKE FROM CELLULOSE DERIVATIVES.

No Drawing.

Application filed March 10, 1922. Serial No. 542,752.

To all whom it may concern:

Be it known that I, HENRY DREYFUS, a citizen of the Swiss Republic, of London, England, have invented certain new and useful Improvements in or Relating to the Manufacture of Artificial Silk and the like from Cellulose Derivatives, of which the following is a specification.

This invention concerns in particular the manufacture of artificial silk or the like from solutions of cellulose acetate, but it may also be applied for the manufacture of artificial filaments and threads from solutions of nitro-cellulose or other cellulose esters, ethers or other derivatives.

The invention relates to what is known as the dry spinning method, that is to say to processes wherein solutions of cellulose acetate, nitrocellulose or other cellulose derivatives in solvents thereof are forced through the fine orifices of jets or spinnerets into the atmosphere to form filaments by evaporation of the solvent or medium, the filaments or threads of associated filaments being wound up on bobbins, hanking-devices or otherwise. In such processes the filaments or threads are sometimes subjected to traction in their travel, for the purpose of drawing them out to greater fineness.

According to the dry spinning method as hitherto proposed the filaments are spun from solutions in solvents of relatively high volatility, such for example as solutions in acetone, methyl acetate and the like.

In spinning with such solutions, the extent to which the solidifying filaments can be drawn out for the production of filaments or threads of low denier is limited, owing to the rapidity with which the filaments issuing from the jets or spinnerets solidify in the heated atmosphere usually employed, low temperatures involving on the other hand too prolonged setting of the filaments for convenient manufacture in practice.

I have now found that by incorporating in the spinning solutions a solvent or solvents of higher boiling points, it is possible to draw the filaments out readily to very fine deniers in dry spinning in a warm or hot atmosphere.

According to the invention I employ in the spinning solutions higher boiling solvents such as referred to, other than tetrachlorethane or such like toxic chlorine derivatives.

The boiling points of the said solvents of

the cellulose acetate or other cellulose derivative will be above that of the acetone or other volatile solvent or liquid used therein and preferably between about 100° C. and 60 about 150-170° C. Solvents of still higher boiling points might be employed in some cases, but usually this is not advantageous, as they would cause the solidification of the filaments to take too long unless relatively 65 high evaporation temperatures were maintained.

Some suitable higher boiling solvents for the purpose of the invention, more particularly in its application with cellulose acetate, are for example acetone-alcohol (acetyl carbinol) b. p. about 147° C., acetylacetone, b. p. about 137° C., cyclopentanone, b. p., about 130° C., diacetone-alcohol b. p. about 163-165° C. and cyclobutanone b. p. 99° C. 75

The higher boiling solvents or solidification retarders used for the invention will be employed together with one or more volatile solvents, such for example as acetone or methyl acetate, and in suitable proportion 80 relatively thereto for the purpose in view. Or organic diluents of lower boiling points than the solidification retarding solvents may be employed instead of or together with the volatile solvent or solvents.

As an example, spinning solutions of cellulose acetate for the purposes of the invention may consist of about 100 parts by weight of cellulose acetate, 400 parts by weight of a volatile solvent for instance 90 acetone, and 25 to 50 parts by weight of higher boiling solvent, for example acetone-alcohol, acetyl acetone, or diacetone-alcohol.

It is to be understood, however, that the constituents and proportions may vary considerably according to circumstances or conditions without departing from the invention.

What I claim and desire to secure by Letters Patent is:—

1. In the dry spinning of artificial threads and filaments from solutions of cellulose derivatives the employment of spinning solutions comprising a volatile solvent and a liquid of a higher boiling point, said liquid 105 of higher boiling point being a solvent of the cellulose derivative, and not being a toxic chlorine derivative, whereby the solidification of the filaments is regulated and the spinning of fine deniers facilitated.

2. In the dry spinning of artificial threads and filaments, the employment of a cellulose

- acetate solution comprising a volatile solvent and a liquid of higher boiling point, said liquid of higher boiling point being a solvent of the cellulose acetate and not being a toxic chlorine derivative, whereby the solidification of the filaments is regulated and the spinning of fine deniers facilitated.
3. A solution for dry spinning artificial threads and filaments, comprising a cellulosic derivative, a volatile solvent and cyclobutanone.
4. A solution for dry spinning artificial threads and filaments, comprising cellulose acetate, a volatile solvent and cyclobutanone.
5. In the manufacture of artificial threads and filaments, dry spinning a solution of cellulose acetate containing a volatile solvent and a solvent of higher boiling point capable of retarding solidification of the filaments and not being a toxic chlorine derivative.
6. In the manufacture of artificial threads and filaments, dry spinning a solution of cellulose acetate containing a volatile solvent and a solvent of higher boiling point lying between about 99° and 170° C., not being a toxic chlorine derivative.
7. In the manufacture of artificial threads and filaments, dry spinning a solution of cellulose acetate containing a volatile solvent and cyclobutanone.
8. In the manufacture of artificial threads and filaments, dry spinning a solution of cellulose derivative containing a volatile solvent and a solvent of higher boiling point capable of retarding solidification of the filaments, and drawing out the filaments during the dry spinning.

In testimony whereof I have hereunto subscribed my name.

HENRY DREYFUS.